

A. S. McDANIEL,  
ANTISTATIC PHOTOGRAPHIC FILM,  
APPLICATION FILED MAR. 26, 1921.

1,431,894.

Patented Oct. 10, 1922.



FIG. 1.



FIG. 2.



WITNESS

*Donald H. Stewart*

Alonzo S. McDaniel,  
INVENTOR

BY *P. L. Stinchfield*

*N. M. Persius*  
ATTORNEYS.

## UNITED STATES PATENT OFFICE.

ALONZO S. McDANIEL, OF NEW YORK, N. Y., ASSIGNOR TO EASTMAN KODAK COMPANY, OF ROCHESTER, NEW YORK, A CORPORATION OF NEW YORK.

## ANTISTATIC PHOTOGRAPHIC FILM.

Application filed March 26, 1921. Serial No. 455,816.

To all whom it may concern:

Be it known that I, ALONZO S. McDANIEL, a citizen of the United States of America, residing at New York, in the county of New York and State of New York, have invented certain new and useful Improvements in Antistatic Photographic Films, of which the following is a full, clear, and exact specification.

10 This invention relates to photographic film. The principal object of this invention is to provide a film having the qualities desirable in commercial practice, which will likewise be so made that markings due to 15 electric discharges are prevented or very greatly minimized.

In the handling of sensitive photographic film, particularly that of the usual kind, which includes a nitrocellulose support or 20 base, characteristic lines or patches sometimes appear on development due to electric discharges which occur when the film is manipulated. While the defect may crop out during manufacture, it is particularly 25 troublesome in the motion picture field, especially when making negative film strips. It is customarily referred to as "static" and will be so designated hereafter.

There have been suggested at different 30 times various methods of combating this evil, among which may be mentioned the application to the back of a film of a soluble gum-like substance, as in British Patent No. 13,088, Mellersh-Jackson, filed June 15, 1913, 35 or the incorporation in the nitrocellulose base of various salts, some of which have hygroscopic properties, this being described in U. S. Patent No. 584,862, Eastman, June 22, 1897, British Patent No. 7501, Boult, filed 40 Apr. 20, 1892, and German Patent No. 69,231, Eastman Photographic Materials Co., Ltd., May 16, 1893. These also describe the use 45 of a metallic salt in a gelatine layer on the back of the film. It may be noted that the gelatine layer would necessarily be more or less softened while wet from the photographic baths. While a gelatine backing is useful in preventing static, one objection to its use on motion picture film is that much 50 of the apparatus ordinarily used in treating film comprises racks, bars and drums which the film passes, or against which it lies during treatment and if the film has a soft backing this becomes objectionably scratched

or marked by such apparatus. It is desirable, therefore, that a backing intended to prevent static on motion picture film should be either entirely removed or substantially unaffected by the photographic baths. In the patent to Lovejoy No. 1,232,702, July 10, 1917, there is described a support for a photographic film in which cellulose acetate and cellulose nitrate are both used, and as there fully set forth, these two substances tend to neutralize each other's tendencies toward the generation of static electricity during the passage of the film over friction surfaces. A support made in accordance with this patent is not affected by the photographic baths.

70 While I have found that film made in the manner described in this patent to be efficient, I have discovered that it is made even more efficient by the introduction of a deliquescent metallic salt into the film base or 75 support.

In order to explain more fully the structure of the film, reference will now be made to the drawings in which:

Fig. 1 is a cross section on a large scale 80 of a photographic film made in accordance with the preferred form of my invention;

Figs. 2, 3 and 4 are similar sections of alternative forms of my invention.

In the drawings, the sensitive layer is indicated as 1. This is carried by a support which comprises both cellulose nitrate and cellulose acetate. These may, if desired, be in two separate layers, the nitrate and acetate being indicated at 2 and 3 respectively 90 in Fig. 1, or they may be incorporated in a common layer as shown at 4 in Fig. 2. The various ways in which this film may be made are fully described in the patent to Lovejoy mentioned. Thus the layer 41 may, as 95 shown in Fig. 3, be a mixture of acetate and nitrate containing the hygroscopic material 1 and 2 representing in this figure respectively the photographically sensitive layer and the nitrocellulose layer, and the nitrocellulose being between the other two. Also

100 the layer 31 in Fig. 4 may be the layer of cellulose acetate containing the hygroscopic material, the photographically sensitive layer being on one side of it, while the nitrocellulose layer 2 is on the other side of it. Of course, the relative thicknesses of 105 the various layers can vary greatly, the di-

mensions in the drawing being exaggerated for the sake of clearness.

In the preferred form of my invention, I incorporate into the material of one of the 5 layers, and preferably that layer containing acetate, a certain amount of hygroscopic material, preferably a deliquescent metallic salt. The particular formula of the "dope" is not essential; many such compositions are 10 known and I contemplate the use of such of these as are referred to in the Lovejoy patent. A salt which I find highly satisfactory is calcium chloride. The quantity of salt introduced into the material of the support 15 may vary within wide limits. A distinctly beneficial effect is observed when to a mass of the dope there is added as little as .05% of calcium chloride. The effect is noticeably better, particularly when from 1% to 2% 20 is used, and I have used as much as 3% with good results. I would consider 3% as about the upper desirable limit of the amount to be used. It is to be noted that in every case the deliquescent salt is incorporated in the 25 material of the support itself, that is to say, in a layer which is a permanent part of the support of the film, and which is for all substantial purposes unaffected and unsoftened by and insoluble in the ordinary 30 photographic baths. This is true even though the layer containing the deliquescent salt is a thin backing layer, and in my preferred form this is the case, the backing layer being the layer containing cellulose 35 acetate. It may be noted that this is to be distinguished from a support containing nitrate only, and also from a support containing a layer such as gelatine or dextrine which will either be softened by or soluble in 40 the developing baths, or from any other layer, whether containing salts or not, deposited on the back surface of the film, which is removed entirely during photographic manipulations.

45 Having thus described my invention, what I claim as new and desire to secure by Letters Patent is:

1. A photographic film comprising a film support, a layer of sensitive material carried thereby and a layer of material which is unsoftened by photographic baths and containing a hygroscopic material.

2. An anti-static photographic film comprising a film support, a layer of sensitive material carried thereby and a backing layer of material insoluble in and unsoftened by photographic baths and containing a deliquescent material.

3. An anti-static photographic film comprising a layer of photographic sensitive material and a support therefor, the support comprising cellulose nitrate and cellulose

acetate and having incorporated therein a deliquescent metallic salt.

4. A photographic film comprising a layer 65 of sensitive material and a support therefor, the support comprising in separate layers two substances respectively adapted to develop positive and negative static charges when acted upon frictionally, one of said 70 layers having incorporated therein hygroscopic material.

5. A photographic film comprising a layer 75 of sensitive material and a support therefor, the support comprising in separate layers two substances respectively adapted to develop positive and negative static charges when acted upon frictionally, one of said 80 layers having incorporated therein a deliquescent metallic salt.

6. A photographic film comprising a layer 85 of sensitive material and a support therefor, the support comprising in separate layers two substances respectively adapted to develop positive and negative static charges when acted upon frictionally, one of said 90 layers having calcium chloride incorporated therein.

7. A photographic film comprising a layer 90 of sensitive material and a support comprising a layer of cellulose nitrate and a layer containing cellulose acetate, one of said layers having a deliquescent metallic salt incorporated therein.

8. An anti-static photographic film comprising a layer of photographically sensitive material, a layer comprising cellulose nitrate and a backing layer containing cellulose acetate, the backing layer containing 95 a deliquescent metallic salt.

9. An anti-static photographic film comprising a layer of photographically sensitive material, a layer comprising cellulose nitrate and a backing layer containing cellulose acetate, the backing layer having calcium chloride incorporated therein. 105

10. An anti-static photographic film comprising a layer of photographically sensitive material, a layer comprising cellulose nitrate, and a backing layer, said backing layer 110 containing cellulose acetate, and having incorporated therein not to exceed 3 per cent of a deliquescent metallic salt.

11. An anti-static photographic film comprising a layer of photographically sensitive material, a layer comprising cellulose nitrate, and a backing layer, said backing layer containing cellulose acetate, and having incorporated therein not to exceed 3 per cent 115 of calcium chloride.

Signed at New York, New York, this 22nd day of March 1921.

ALONZO S. McDANIEL.